# EUROPEAN PATENT APPLICATION

(11) **EP 0 558 311 A1**
(43) Date of publication of application: **01.09.1993**
(21) Application number: 93301392.2
(22) Date of filing: 24.02.1993
(51) Int. Cl.: B41N 3/03

(54) **Light-sensitive lithographic printing plate**

(30) Priority: 26.02.1992 JP 75177/92
(71) Applicant: KONICA CORPORATION, Tokyo 163 (JP); Mitsubishi Chemical Corporation, Chiyoda-ku Tokyo (JP)
(72) Inventor: Matsubara, Shinichi, Hino-shi, Tokyo (JP); Tomita, Yasuji, Hino-shi, Tokyo (JP); Nakai, Hideyuki, Hino-shi, Tokyo (JP); Naito, Kunitaka, Sakura-shi, Chiba-ken (JP); Tsuchiya, Tatsunori, Kashima-gun, Ibaraki-ken (JP); Nishizawa, Hiroyuki, Kashima-gun, Ibaraki-ken (JP)
(74) Representative: Brock, Peter William

(57) **Abstract**

Disclosed is a light-sensitive lithographic printing plate which comprises a support being treated by a process comprising steps of neutralizing electric charge of a surface of a pre-treated support; and treating said neutralized support with a hydrophilic polymer aqueous solution, and a light-sensitive layer provided on the support.

## Description

### BACKGROUND OF THE INVENTION

This invention relates to a light-sensitive lithographic printing plate, particularly to a light-sensitive lithographic printing plate having an improved support.

In the prior art, as a support used for a lithographic printing plate, an aluminum plate has been generally used from the points of hydrophilicity, water retention and adhesiveness to a light-sensitive layer.

However, the prior art lithographic printing plate using the above support is insufficient to satisfy the requirements of stain-preventing property at a non-image portion as well as press life and chemical resistance, simultaneously. In order to solve such a problem, in Japanese Provisional Patent Publication No. 289388/1990, there has been proposed a method in which the surface of a pretreated support is treated with an aqueous solution containing nitrous acid or an nitrite.

However, even in the method described above, stain at a non-image portion cannot be prevented sufficiently, so that fingerprint marks may be left or an ink component contained in a stained dampening water may be attached to a non-image portion. Thus, it is difficult to obtain a printed matter having no stain stably. The method is also insufficient in the point of loss of printing papers at the beginning of printing, which is caused by gum removability.

### SUMMARY OF THE INVENTION

An object of the present invention is to provide a light-sensitive lithographic printing plate in which press life is excellent, stain at a non-image portion can be prevented and printing stain caused by fingerprint marks or the like can be prevented.

Another object of the present invention is to provide a light-sensitive lithographic printing plate which can reduce loss of printing papers at the beginning of printing.

The present inventors have studied intensively in consideration of the above tasks, and consequently found that the above objects of the present invention can be accomplished by (a) a light-sensitive lithographic printing plate which comprises a support being treated by a process comprising steps of neutralizing electric charge of a surface of a pre-treated support; and treating said neutralized support with a hydrophilic polymer aqueous solution, and a light-sensitive layer provided on the support, more specifically (a') the above light-sensitive lithographic printing plate treated with a hydrophilic polymer aqueous solution comprising 1 % by weight or less of a hydrophilic polymer and having a pH value of 9 or less and a temperature of 60 °C or higher and (b) a light-sensitive lithographic printing plate which comprises a support being treated by a process comprising steps of neutralizing electric charge of a surface of a pre-treated support with nitrous acid and/or a nitrite; and treating said neutralized support with hot water before treating it with a hydrophilic polymer aqueous solution, and a light-sensitive layer provided on the support.

### DESCRIPTION OF THE PREFERRED EMBODIMENTS

In the following, the present invention is explained in detail.

The neutralization of electric charge of the surface of a support in the present invention means that electric charge is neutralized to a degree that a support is not dyed by a dyeing test described below. The present inventors have found that electric charge of the surface of a support is one of the factors which exert great influences on attachment of polar components such a dye and an alkali-soluble polymer compound in a light-sensitive layer provided on said surface, and when the surface of a support has positive electric charge, a part of a light-sensitive composition remains on the surface of an image portion obtained by development processing, whereby the surface of a non-image portion is easily stained. Thus, it is suitable that electric charge on the surface of a support is neutralized, and the neutralization degree of electric charge is preferably a degree that a support is not dyed by a dyeing test described below.

The dyeing test in the present invention is carried out by dipping a support in an aqueous solution containing a 0.05 to 10 % by weight of an acidic dye having negative electric charge at room temperature for 0.5 to 5 minutes, then washing and drying the support and observing a dyeing result of a dipped portion of the support visually with naked eyes or by an optical reflection densitometer.

As the acidic dye having negative electric charge to be used in the present invention, there may be used conventionally known dyes such as Orange II (trade name, produced by Wako Junyaku K.K.), Naphthol Yellow S, Tartrazine, Acid Fast Orange SG, Eosine G, Acid Milling Red RS, Alizarine Direct Blue AGG, Indigo Carmine Blue G, Acid Milling Cyanine 5R, Brilliant Milling Green B, Acid Cyanine Green G, Acid Fast Brown R, Acid Blue Black 10B and Acid Milling Black VLG.

As a method for obtaining the neutralized support, various methods can be used, and preferred is a method of treating with an aqueous solution containing nitrous acid and/or a nitrite or a method of treating with an aqueous solution containing at least one of the compounds represented by the formulae (I) to (III) shown below.

As an example of the nitrite to be used in the present invention, there may be mentioned a nitrite of a metal of the Ia, IIa, IIIa, IVa, VIa, VIIa, VIII, IIb, IIIb and IVb group of the periodic table, or ammonium nitrite. As such a metal salt, preferred are, for example, LiNO₂, NaNO₂, KNO₂, Mg(NO₂)₂, Ca(NO₂)₂, Zn(NO₂)₂, Al(NO₂)₃, Zr(NO₂)₄, Sn(NO₂)₄, Cr(NO₂)₃, Co(NO₂)₂, Mn(NO₂)₂ and Ni(NO₂)₂, and particularly preferred is an alkali metal nitrite. The above nitrites may be used in combination of two or more, and may be further used in combination with nitrous acid.

The aqueous solution containing nitrous acid and/or the nitrite to be used in the present invention is preferably an aqueous solution containing 0.001 to 10 % by weight of nitrous acid and/or the nitrite.

As treatment conditions for treating the surface of a support with the above treating solution, it is preferred that a pre-treated support is dipped in the treating solution for 3 to 300 seconds at a temperature range between room temperature and about 100 °C, or the treating solution is coated on a support.

As a preferred embodiment of the present invention, there may be mentioned a treatment in which a support is dipped in an aqueous solution containing 0.01 to 2 % by weight of sodium nitrite at 50 to 90 °C for 3 to 180 seconds. The support treated with the aqueous solution containing nitrous acid and/or the nitrite is preferably followed by drying.

To the above aqueous solution containing nitrous acid and/or a nitrite, an additive may be added, if necessary As the additive, there may be mentioned, for example, a water-soluble polymer and a surfactant.

As the support to be used in the present invention, there may be preferred a support which is flexible enough to be set in a conventional lithographic printing machine and can stand load applied during printing, and there may be mentioned, for example, a plate of a metal such as aluminum, magnesium, zinc, iron containing chronium and copper containing nickel, and a plate of an alloy of these metals. Further, a metal plate coated with chromium, zinc, copper, nickel, aluminum or iron by plating or vapor deposition may be used. Among them, a preferred support is aluminum or an alloy thereof.

The support to be used in the present invention is subjected to pre-treatment before treatment with the aqueous solution containing nitrous acid and/or a nitrite. The pre-treatment includes degreasing treatment and graining treatment conventionally utilized in this field of the art.

The degreasing treatment is treatment of washing the support with an alkaline aqueous solution such as a sodium hydroxide aqueous solution in order to remove an oil film of the surface of the support.

The graining treatment is mechanical roughening of a surface and called the mechanical roughening method, and may include, for example, methods such as ball grinding, brush grinding, blast grinding and buff grinding. Also, the so-called electrical roughening method in which a surface is roughened electrically may be utilized. For example, a support may be also subjected to electrolysis treatment in an electrolyte containing hydrochloric acid or nitric acid by an alternating current or direct current.

On the surface of the support obtained by graining treatment as described above, smut is generated. In order to remove the smut, it is generally preferred to carry out suitable treatment such as washing or alkaline etching. As such a treatment, there may be mentioned, for example, the alkaline etching method described in Japanese Patent Publication No. 28123/1973 and the sulfuric acid desmutting method described in Japanese Provisional Patent Publication No. 12739/1978.

When the support to be used in the present invention is an aluminum support, after the pre-treatment as described above is carried out, an oxidized layer is generally formed on the surface of the support by anodization in order to improve abrasion resistance, chemical resistance and water retention. As the anodization, there may be generally preferably used a method in which electrolysis is effected at a current density of 1 to 10 A/dm² by using an aqueous solution containing 10 to 50 % sulfuric acid and/or phosphoric acid as an electrolyte. Also, there may be used a method in which electrolysis is effected in sulfuric acid at a high current density described in U.S. Patent No. 1,412,768 and a method in which electrolysis is effected by using phosphoric acid described in U.S. Patent No. 3,511,661.

The most preferred support to be used in the present invention is an aluminum support having an anodized layer.

The support treated with the aqueous solution containing nitrous acid and/or a nitrite described above is then treated with a hydrophilic substance and/or polymer aqueous solution (in the specification, the hydrophilic polymer aqueous solution also includes a hydrophilic substance aqueous solution even when it is not referred to). As a preferred hydrophilic substance and a hydrophilic polymer to be used in the hydrophilic polymer aqueous solution, there may be mentioned an acrylic acid copolymer such as polyacrylic acid, polyacrylamide, polyvinyl alcohol, polyhydroxyethyl acrylate and polyvinyl pyrrolidone; a maleic acid copolymer such as polyethyleneimine, diacryldimethyl ammonium chloride, polyvinylimidazoline and polyalkylaminoethyl acrylate; a water-soluble substance or polymer such as polyethylene glycol polyoxyethylene, polypropylene glycol, ethylenediamine, hexaethylenediamine, a polyurethane resin, a polyhydroxymethyl urea, a polyhydroxymethyl melamine resin, a soluble starch, CMC (carboxymethyl cellulose), hydroxyethyl cellulose, guar gum, tragacanth gum, xanthane gum, sodium alginate and gelatin.

The hydrophilic polymer aqueous solution in the present invention is an aqueous solution containing 1 % by weight or less, preferably 0.001 to 0.1 % by weight of the above hydrophilic polymer. The hydrophilic polymer aqueous solution preferably has a pH value of 9 or less, preferably 6 to 9 or a temperature of 60 °C or higher, preferably 70 to 95 °C. It is particularly preferred that the hydrophilic polymer aqueous solution satisfies both of these conditions. The support is contacted with the hydrophilic polymer aqueous solution for 1 second to 3 minutes, preferably 1 second to 1 minute.

In the present invention, it is preferred that the support is treated with nitrous acid and/or the nitrite described above, then treated with hot water before being treated with a hydrophilic polymer aqueous solution. Such a hot water treatment is preferably carried out under conditions of a pH value or 9 or less, preferably 6 to 9 or a temperature of 60 °C or higher, preferably 70 to 95 °C, particularly preferably carried out under conditions satisfying both of the pH value and temperature range described above. The support is contacted with hot water for 1 second to 3 minutes, preferably 1 second to 1 minute. For the purposes of pH adjustment and others, the hot water may optionally contain a compound such as NaOH, KOH, NaHCO₃, NH₃, Ca(OH)₂, KHCO₃, Ba(OH)₂, CaO, MgO, CaCO₃, NaCO₃, Fe(OH)₃, Al(OH)₃ and CH₃COONa.

In the present invention, the neutralized support is also obtained by treating with a carboxylate represented by any of the following formulae:

(R¹COO)ₙX¹ (I)

wherein n represents 1 or 2; when n is 1, R¹ represents a hydrogen atom, an aliphatic hydrocarbon group having 1 to 10 carbon atoms, an alicyclic hydrocarbon group or an aromatic hydrocarbon group and X¹ represents NH₄⁺ or an alkali metal ion; and when n is 2, R¹s may be the same or different and each represent a hydrogen atom, an aliphatic hydrocarbon group having 1 to 10 carbon atoms, an alicyclic hydrocarbon group or an aromatic hydrocarbon group and X¹ represents a monovalent or divalent metal ion selected from the group consisting of metal ions of the Ia (excluding a hydrogen ion), IIa, VIIa, VIII, IIb and IVb groups of the periodic table,
wherein R² represents a direct bond, or a divalent aliphatic hydrocarbon group having 1 to 10 carbon atoms, a divalent alicyclic hydrocarbon group or a divalent aromatic hydrocarbon group; and X² and X³ may be the same or different and each represent NH₄⁺ or an alkali metal ion, or a monovalent or divalent metal ion selected from the group consisting of metal ions of the Ia (excluding a hydrogen ion), IIa, VIIa, VIII, IIb and IVb groups of the periodic table,

R³(COO)₂X⁴ (III)

wherein R³ represents a direct bond, or a divalent aliphatic hydrocarbon group having 1 to 10 carbon atoms, alicyclic hydrocarbon group or aromatic group; and X⁴ represents a monovalent or divalent metal ion selected from the group consisting of metal ions of the Ia (excluding a hydrogen ion), IIa, VIIa, VIII, IIb and IVb groups of the periodic table.

The compound is preferably a hydrophilic compound containing at least one of the compounds having the following structures:
wherein R¹, R², R³, X¹, X², X³ and X⁴ each have the same meanings as defined above.

In the above formulae (I), (II) and (III), it is preferred that R¹ represents a hydrogen atom or an alkyl group having 1 to 4 carbon atoms; X¹ represents NH₄⁺, an alkali metal ion of sodium, potassium or lithium, or a monovalent or divalent metal ion of calcium, barium, magnesium, zinc, manganese, nickel, strontium or lead; R² represents a direct bond or an alkylene group or phenylene group having 1 to 4 carbon atoms; X² and X³ each represent a hydrogen atom, NH₄⁺ or an alkali metal ion of sodium, potassium or lithium; R³ represents a direct bond or an alkylene group or phenylene group having 1 to 4 carbon atoms; and X⁴ represents a monovalent or divalent metal ion of calcium, barium, magnesium, zinc, manganese, nickel, strontium of lead.

Among these compounds, as the useful compound to be used in the present invention, there may be mentioned ammonium formate, sodium formate, potassium formate, lithium formate, calcium formate, barium formate, magnesium formate, zinc formate, manganese formate, nickel formate, strontium formate, lead formate, ammonium acetate, sodium acetate, potassium acetate, lithium acetate, calcium acetate, barium acetate, magnesium acetate, zinc acetate, manganese acetate, nickel acetate, strontium acetate, lead acetate, ammonium propionate, sodium propionate, potassium propionate, lithium propionate, calcium propionate, barium propionate, magnesium propionate, zinc propionate, manganese propionate, nickel propionate, strontium propionate, lead propionate, ammonium butyrate, sodium butyrate, potassium butyrate, lithium butyrate, calcium butyrate, barium butyrate, magnesium butyrate, zinc butyrate, manganese butyrate, nickel butyrate, strontium butyrate, lead butyrate, ammonium oxalate, ammonium hydrogen oxalate, sodium oxalate, sodium hydrogen oxalate, potassium oxalate, potassium hydrogen oxalate, lithium oxalate, lithium hydrogen oxalate, calcium oxalate, barium oxalate, magnesium oxalate, zinc oxalate, manganese oxalate, nickel oxalate, strontium oxalate, lead oxalate, ammonium malonate, ammonium hydrogen malonate, sodium malonate, sodium hydrogen malonate, potassium malonate, potassium hydrogen malonate, lithium malonate, lithium hydrogen malonate, calcium malonate, barium malonate, magnesium malonate, zinc malonate, manganese malonate, nickel malonate, strontium malonate, lead malonate, ammonium succinate, sodium succinate, potassium succinate, lithium succinate, calcium succinate, barium succinate, magnesium succinate, zinc succinate, manganese succinate, nickel succinate, strontium succinate, lead succinate, ammonium glutarate, sodium glutarate, potassium glutarate, lithium glutarate, calcium glutarate, barium glutarate, magnesium glutarate, zinc glutarate, manganese glutarate, nickel glutarate, strontium glutarate, lead glutarate, ammonium phthalate, sodium phthalate, potassium phthalate, lithium phthalate, calcium phthalate, barium phthalate, magnesium phthalate, zinc phthalate, nickel phthalate, strontium phthalate and lead phthalate.

The hydrophilic compound as described above is dissolved in a suitable solvent, for example, water or an alcohol such as methanol so as to have a concentration of 0.001 to 10 % by weight, to prepare a coating solution. Here, the pH value after coating is suitably in the range of 1 to 13. Further, the temperature of the coating solution is suitably in the range of 10 to 50 °C.

As a coating method, there may be used any method such as dip coating, rotational coating, spray coating and curtain coating. The amount to be coated is preferably in the range of 1 to 100 mg/m², more preferably 5 to 50 mg/m² in terms of a coated amount after drying.

After treatment with the aqueous solution as described above, the support is treated with the above hydrophilic polymer aqueous solution.

In the light-sensitive lithographic printing plate of the present invention, a primer layer may be provided on the above support, if necessary, in order to improve adhesiveness of the above support to a light-sensitive layer.

As the primer layer, there may be used, for example, a polyester resin, a vinyl chloride-vinyl acetate copolymer, an acryl resin, a vinyl chloride resin, a polyamide resin, a polyvinyl butyral resin, an epoxy resin, an acrylate type copolymer, a vinyl acetate type copolymer, a phenoxy resin, a polyurethane resin, a polycarbonate resin, a polyacrylo-nitrile-butadiene and a polyvinyl acetate.

As an anchoring agent constituting the above primer layer, there may be used, for example, a silane coupling agent and a silicone primer, and an organic titanate is also effective.

The light-sensitive lithographic printing plate of the present invention comprises a light-sensitive layer provided on the support obtained as described above. A light-sensitive substance to be used in the light-sensitive layer is not particularly limited, and may include, for example, the following composition conventionally used in a light-sensitive lithographic printing plate.

Light-sensitive composition containing o-quinonediazide compound

In the light-sensitive composition containing an o-quinonediazide compound, an o-quinonediazide compound and an alkali-soluble resin are preferably used in combination.

As the o-quinonediazide compound, there may be mentioned, for example, an ester compound of o-naphthoquinonediazide-sulfonic acid and a polycondensed resin of a phenol and an aldehyde or a ketone.

As the above phenol, there may be mentioned, for example, a monovalent phenol such as phenol, o-cresol, m-cresol, p-cresol, 3,5-xylenol, carvacrol and thymol; a divalent phenol such as catechol, resorcin and hydroquinone; and a trivalent phenol such as pyrogallol and phloroglucin. The above aldehyde may include formaldehyde, benzaldehyde, actaldehyde, crotonaldehyde and furfural. Among them, preferred are formaldehyde and benzaldehyde. Further, the above ketone may include acetone and methyl ethyl ketone.

As a specific example of the above polycondensed resin, there may be mentioned a phenol·formaldehyde resin, an m-cresol·formaldehyde resin, an m- and p-mixed cresol·formaldehyde resin, a resorcin-benzaldehyde resin and a pyrogallol·acetone resin.

In the above o-naphthoquinonediazide compound, the condensation ratio of o-naphthoquinonediazidesulfonic acid to an OH group of the phenol (reactivity based on one OH group) is preferably 15 to 80 %, more preferably 20 to 45 %.

As the o-quinonediazide compound to be used in the present invention, there may be also used the following compounds described in Japanese Provisional Patent Publication No. 43451/1983, for example, conventionally known 1,2-quinonediazide compounds such as 1,2-benzoquinonediazidesulfonate, 1,2-naphthoquinonediazidesulfonate, 1,2-benzoquinonediazidesulfonic acid amide and 1,2-naphthoquinonediazidesulfonic acid amide. More specifically, there may be mentioned 1,2-quinonediazide compounds such as phenyl 1,2-benzoquinonediazide-4-sulfonate, 1,2,1',2'-di-(benzoquinonediazide-4-sulfonyl)-dihydroxybiphenyl, 1,2-benzoquinonediazide-4-(N-ethyl-N-β-naphthyl)-sulfonamide, cyclohexyl 1,2-naphthoquinonediazide-5-sulfonate, 1-(1,2-naphthoquinonediazide-5-sulfonyl)-3,5-dimethylpyrazole, 1,2-naphthoquinonediazide-5-sulfonic acid-4'-hydroxydiphenyl-4'-azo-β-naphthol ester, N,N-di-(1,2-naphthoquinonediazide-5-sulfonyl)-aniline, 2'-(1,2-naphthoquinonediazide-5-sulfonyloxy)-1-hydroxy-anthraquinone, 1,2-naphthoquinonediazide-5-sulfonic acid-2,4-dihydroxybenzophenone ester, 1,2-naphthoquinonediazide-5-sulfonic acid-2,3,4-trihydroxybenzophenone ester, a condensate of 2 mole of 1,2-naphthoquinonediazide-5-sulfonic acid chloride and 1 mole of 4,4'-diaminobenzophenone, a condensate of 2 mole of 1,2-naphthoquinonediazide-5-sulfonic acid chloride and 1 mole of 4,4'-dihydroxy-1,1'-diphenylsulfone, a condensate of 1 mole of 1,2-naphthoquinonediazide-5-sulfonic acid chloride and 1 mole of purpurogallin and 1,2-naphthoquinonediazide-5-(N-dihydroabietyl)-sulfonamide described in J. Kosar, "Light-Sensitive Systems", pp. 339 to 352 (1965), John Wiley & Sons Co. (New York) and W.S. De Forest, "Photoresist", Vol. 50 (1975), McGraw-Hill Co. (New York). Also, there may be mentioned 1,2-quinonediazide compounds described in Japanese Patent Publications No. 1953/1962, No. 3627/1962, No. 13109/1962, No. 26126/1965, No. 3801/1965, No. 5604/1970, No. 27345/1970 and No. 13013/1976, and Japanese Provisional Patent Publications No. 96575/1973, No. 63802/1973 and No. 63803/1973.

Among the o-quinonediazide compounds described above, particularly preferred is an o-quinonediazide ester compound obtained by reacting 1,2-benzoquinonediazidesulfonyl chloride or 1,2-naphthoquinonediazidesulfonyl chloride and a pyrogallol·acetone condensed resin or 2,3,4-trihydroxybenzophenone.

As the o-quinonediazide compound to be used in the present invention, the above compounds may be used singly or in combination of two or more.

The ratio of the o-quinonediazide compound to be used in the present invention in the light-sensitive composition is preferably 5 to 60 % by weight, particularly preferably 10 to 50 % by weight.

As the alkali-soluble resin to be used in the light-sensitive lithographic printing plate of the present invention, there may be mentioned a novolak resin, a vinyl type polymer having a phenolic hydroxyl group and a condensed resin of a polyvalent phenol and an aldehyde or a ketone described in Japanese Provisional Patent Publication No. 57841/1980.

As the novolak resin to be used in the present invention, there may be mentioned, for example, a phenol·formaldehyde resin, a cresol·formaldehyde resin, a phenol·cresol·formaldehyde copolycondensed resin as described in Japanese Provisional Patent Publication No. 57841/1980 and a copolycondensed resin of p-substituted phenol and phenol or cresol and formaldehyde as described in Japanese Provisional Patent Publication No. 127553/1980.

As to the molecular weight (based on polystyrene) of the above novolak resin, the number average molecular weight Mn is preferably 3.00 x 10² to 7.50 x 10³, and the weight average molecular weight Mw is 1.00 x 10³ to 3.00 x 10⁴. It is more preferred that Mn is 5.00 x 10² to 4.00 x 10³, and Mw is 3.00 x 10³ to 2.00 x 10⁴.

The above novolak resins may be used singly or in combination of two or more.

The ratio of the above novolak resin in the light-sensitive composition of the present invention is 5 to 95 % by weight.

The vinyl type polymer having a phenolic hydroxyl group to be used in the present invention is a polymer containing a unit having said phenolic hydroxyl group in a molecular structure, preferably a polymer containing at least one of the constitutional units of the formulae (1) to (5) shown below:
wherein R₁ and R₂ each represent a hydrogen atom, an alkyl group or a carboxyl group, preferably a hydrogen atom; R₃ represents a hydrogen atom, a halogen atom or an alkyl group, preferably a hydrogen atom or an alkyl group such as a methyl group and an ethyl group; R₄ represents a hydrogen atom, an alkyl group, an aryl group or an aralkyl group, preferably a hydrogen atom; A represents a substituted or unsubstituted alkylene group linking a nitrogen atom or an oxygen atom and an aromatic carbon atom; m represents an integer of 0 to 10; and B represents a phenylene group which may have a substituent(s) or a naphthylene group which may have a substituent(s).

The polymer to be used in the light-sensitive composition of the present invention preferably has a copolymer type structure. As a monomer unit which can be used in combination with the constitutional units represented by the above formulae (1) to (5), respectively, there may be mentioned vinyl type monomers including ethylenic type unsaturated olefins such as ethylene, propylene, isobutylene, butadiene and isoprene; styrenes such as styrene, α-methylstyrene, p-methylstyrene and p-chlorostyrene; acrylic acids such as acrylic acid and methacrylic acid; unsaturated aliphatic dicarboxylic acids such as itaconic acid, maleic acid and maleic anhydride; esters of α-methylene aliphatic monocarboxylic acid such as methyl acrylate, ethyl acrylate, n-butyl acrylate, isobutyl acrylate, dodecyl acrylate, 2-chloroethyl acrylate, phenyl acrylate, methyl α-chloroacrylate, methyl methacrylate, ethyl methacrylate and ethyl ethacrylate; nitriles such as acrylonitrile and methacrylonitrile; amides such as acrylamide; anilides such as acrylanilide, p-chloroacrylanilide, m-nitroacrylanilide and m-methoxyacrylanilide; vinyl esters such as vinyl acetate, vinyl propionate, vinyl benzoate and vinyl butyrate; vinyl ethers such as methyl vinyl ether, ethyl vinyl ether, isobutyl vinyl ether and β-chloroethyl vinyl ether; vinyl chloride; vinylidene chloride; vinylidene cyanide; ethylene derivatives such as 1-methyl-1-methoxyethylene, 1,1-dimethoxyethylene, 1,2-dimethoxyethylene, 1,1-dimethoxycarbonylethylene and 1-methyl-1-nitroethylene; and N-vinyl compounds such as N-vinylpyrrole, N-vinylcarbazole, N-vinylindole, N-vinylpyrrolidene and N-vinylpyrrolidone. These vinyl type monomers exist in polymer compounds in a structure of a cleaved double bond.

Among the monomers described above, preferred are esters of aliphatic monocarboxylic acid and nitriles which show excellent characteristics to obtain the effect of the present invention.

These monomers may be bonded in the polymer of the present invention either in a block state or in a random state.

The ratio of the vinyl type polymer to be used in the present invention in the light-sensitive composition is 0.5 to 70 % by weight.

The vinyl type polymers to be used in the present invention may be used singly or in combination of two or more. Further, they may be also used in combination with other polymer compounds.

To the light-sensitive lithographic printing plate of the present invention, a print-out material which forms a visible image by exposure may be added. The print-out material comprises a compound which forms an acid or a free group by exposure and an organic dye which changes its color tone by interaction with said compound. As the compound which forms an acid or a free group by exposure, there may be mentioned, for example, o-naphthoquinonediazide-4-sulfonic acid halogenide described in Japanese Provisional Patent Publication No. 36209/1975, trihalomethyl-2-pyrone and trihalomethyl-triazine described in Japanese Provisional Patent Publication No. 36223/1978, an ester compound or an amide compound comprising o-naphthoquinonediazide-4-sulfonic acid chloride and a phenol having an electron-attracting substituent or anilic acid described in Japanese Provisional Patent Publication No. 6244/1980, and a halomethylvinyloxadiazole compound and a diazonium salt described in Japanese Provisional Patent Publications No. 77742/1980 and No. 148784/1984.

As the above organic dye, there may be mentioned Victoria Pure Blue BOH (trade name, produced by Hodogaya Kagaku K.K.), Patent Pure Blue (trade name, produced by Sumitomo Mikuni Kagaku K.K.), Oil Blue #603 (trade name, produced by Orient Kagaku Kogyo K.K.), Sudan Blue II (trade name, produced by BASF), Crystal Violet, Malachite Green, Fuchsin, Methyl Violet, Ethyl Violet, Methyl Orange, Brilliant Green, Congo Red, Eosin and Rhodamine 6G. To the light-sensitive composition, in addition to the materials described above, a plasticizer, a surfactant, an organic acid and an acid anhydride may be added, if necessary.

To the light-sensitive lithographic printing plate of the present invention, for example, a p-tert-butylphenolformaldehyde resin, a p-n-octylphenolformaldehyde resin or a resin in which the above resin is partially esterified with an o-quinonediazide compound may be further added in order to improve ink receptivity of the light-sensitive composition.

The light-sensitive lithographic printing plate of the present invention can be prepared by dissolving these respective components in a solvent described below and coating the resulting solution on the surface of the support of the present invention, followed by drying to provide a light-sensitive layer on the support.

As the solvent which can be used for dissolving the above respective components, there may be mentioned methyl cellosolve, methyl cellosolve acetate, ethyl cellosolve, ethyl cellosolve acetate, diethylene glycol monomethyl ether, diethylene glycol monoethyl ether, diethylene glycol dimethyl ether, diethylene glycol methyl ethyl ether, diethylene glycol diethyl ether, dimethyl glycol monoisopropyl ether, propylene glycol, propylene glycol monomethyl ether acetate, propylene glycol monoethyl ether acetate, propylene glycol monobutyl ether, dipropylene glycol monomethyl ether, dipropylene glycol dimethyl ether, dipropylene glycol methyl ethyl ether, ethyl formate, propyl formate, butyl formate, amyl formate, methyl acetate, ethyl acetate, propyl acetate, butyl acetate, methyl propionate, ethyl propionate, methyl butyrate, ethyl butyrate, dimethylformamide, dimethylsulfoxide, dioxane, acetone, methyl ethyl ketone, cyclohexanone, methylcyclohexanone, diacetone alcohol, acetylacetone and γ-butyrolactone. These solvents may be used singly or in combination of two or more.

As a coating method used for coating the light-sensitive composition to be used in the present invention on the surface of the support, there may be used a conventionally known method, for example, rotational coating, wire bar coating, dip coating, air knife coating, roll coating, blade coating and curtain coating. The amount to be coated varies depending on the use, but may be preferably, for example, 0.05 to 5.0 g/m² as a solid component.

The light-sensitive lithographic printing plate thus obtained can be used according to a conventionally used method. For example, a transparent original picture having a line image or a dot image is closely contacted to a light-sensitive surface and subjected to exposure, and then a light-sensitive layer at a non-image portion is removed by using a suitable developing solution to obtain a relief image. As a suitable light source for exposure, there may be used a mercury lamp, a metal halide lamp, a xenon lamp, a chemical lamp and a carbon arc lamp.

As the developing solution to be used for development, preferred is an alkaline aqueous solution and the alkaline aqueous solution may include an aqueous solution of sodium silicate, potassium silicate, sodium hydroxide, potassium hydroxide, sodium tertiary phosphate, sodium secondary phosphate, sodium carbonate or potassium carbonate. The concentration of the alkaline aqueous solution varies depending on the light-sensitive composition and the kind of an alkali, but may be generally suitably in the range of 0.1 to 10 % by weight. Further, to said alkaline aqueous solution, a surfactant and an organic solvent such as alcohol may be added, if necessary.

### EXAMPLES

The present invention is described in detail by referring to Examples.

### Example 1

### Preparation of Supports-1 to 5

An aluminum plate (material: 1050, tempering: H16) having a thickness of 0.3 mm was degreased in a 5 % sodium hydroxide aqueous solution at 65 °C for 1 minute, washed, dipped in a 10 % nitric acid aqueous solution at 25 °C for 1 minute, neutralized and then washed.

Next, the plate was electrolytically roughened in a 0.5N hydrochloric acid aqueous solution at 25 °C at an alternate current density of 55 A/dm² for 35 seconds and then desmutted in a 5 % sodium hydroxide aqueous solution at 60 °C for 10 seconds.

Thereafter, the plate was anodized in a 20 % sulfuric acid solution under conditions of a temperature of 20 °C, a current density of 3 A/dm² and a treatment time of 1 minute, and washed.

The aluminum plate having been subjected to the above treatments was dipped in aqueous solutions having the following compositions at 80 °C for 1 minute, and then dipped in a 0.005 % CMC aqueous solution at 80 °C for 1 minute to prepare Supports-1 to 5.

| | |
|---|---|
| Support-1 | 1 % Sodium nitrite |
| Support-2 | 1 % Potassium nitrite |
| Support-3 | 1 % Calcium nitrite |
| Support-4 | 1 % Ammonium nitrite |
| Support-5 | 1% Nickel nitrite |

### Preparation of Light-sensitive lithographic printing plates I-1 to I-5

On Supports-1 to 5 prepared as described above, a light-sensitive composition coating solution (1) having the following composition was coated by using a wire bar, respectively, and dried at 80 °C for 2 minutes. The coated film thickness was 2.2 g/m².

### (Composition of light-sensitive composition coating solution (1))

### Novolak resin A

A copolycondensed resin of phenol, m-cresol, p-cresol and formaldehyde (molar ratio of phenol, m-cresol and p-cresol: 2.0:4.8:3.2, Mw = 6500, Mw/Mn = 5.4)

### o-Quinonediazide compound B

### Surfactant C

Emulgen 120 (trade name, produced by Kao K.K.), polyoxyethyl lauryl ether

### Compound D forming a halogen free group

2-Trichloromethyl-5-(p-methoxystyryl)-1,3,4-oxadiazole (a compound described in Example 1 of Japanese Provisional Patent Publication No. 74728/1979)

The respective light-sensitive lithographic printing plate samples obtained were exposed at 8 mW/cm² for 60 seconds by using a 2 kw metal halide lamp, and developed for a developing time of 30 seconds at a developing temperature of 25 °C by using a 5-fold diluted solution of a commercially available developing solution SDR-1 (trade name, produced by Konica Corporation) to obtain Lithographic printing plate samples I-1 to I-5.

For the samples obtained, dyeing by Orange II (trade name, produced by Wako Junyaku K.K.), stain caused by a remaining photosensitive layer, resistance to chemical for printing plate, dot reproducibility and a number of lost printing papers were evaluated. The results are shown in Table 1.

### Evaluation methods

### Test of stain caused by remaining photosensitive layer

On the lithographic printing plates obtained by the exposure and development conditions described above, 5 lines (5 mm x 15 cm) of image portions were formed, and the image portions were removed by using Image remover SIR-15 (trade name, produced by Konica Corporation). The image portions were removed for 5 kinds of removing times (shown in Table 1), and fringe stain caused by removing was inked by a developing ink SPO-1 (trade name, produced by Konica Corporation).

### Evaluation standard

- ○:: Good (no fringe stain)
- Δ:: An removed mark appears. (not inked, but a remaining photosensitive layer can be clearly confirmed visually with naked eyes)
- X:: Stained

### Resistance to chemical for printing plate

The samples obtained by the exposure and development conditions described above were dipped in inks SPO-1 (trade name, produced by Konica Corporation) and PI (trade name, produced by Fuji Photo Film K.K.) for development inking and a plate cleaner UPC (trade name, produced by ABC Chemical Co.) used at the time of printing for predetermined times, respectively, and the state of image on each plate was evaluated by the following standard.

### Evaluation standard

- ○:: No change
- Δ:: The surface of a solid portion is corroded.
- X:: A solid portion is peeled off.

### Dot reproducibility

By using the lithographic printing plates obtained by the above method, printing was carried out in a printing machine Heidelberg GTO (trade name, produced by Heidelberger Druckinaschinen AG (Germany)) by using a coated paper-printing ink New Bright Magenta (trade name, produced by Toyo Ink Seizo K.K.) and a plate etch aqueous solution SEU-3 (2.5 %, trade name, produced by Konica Corporation). For the printed papers obtained, dot reproducibility at a large dot portion (dot area ratio: 97 %) of a dot image was evaluated by using a loupe of 25 magnifications according to the following standard.

### Evaluation standard

- ○:: Reproduced (no entanglement)
- X:: Not reproduced (entanglement exists)

### Press life

Under the printing conditions as described above, printing was continued until inking failure was caused at a solid image portion of a printed paper or inked on a non-image portion, and a number of printed papers until then was counted.

### Loss of printing papers (gum removability)

Printing was carried out under the same conditions as in the evaluation of dot reproducibility. A number of printed papers until stain on printed papers by gum disappeared completely was counted and designated as a number of lost papers.

### Dyeing test by Orange II (trade name)

The sample was dipped in an aqueous solution containing 0.2 % Orange II (trade name, produced by Wako Junyaku K.K.) at 20 °C for 1 minute after treatment with the nitrite and before treatment with the CMC aqueous solution, then washed with running water and dried. Then, coloring degree of the dipped portion was evaluated visually with naked eyes. Further, reflection densities of the surface of the sample before dipping and after dipping were measured by a green filter of Sakura Densitometer PDA 65 (trade name, manufactured by Konica Corporation) to determine difference in the reflection densities before dipping and after dipping.

### Comparative example 1

### Preparation of Supports-6 to 10

Supports-6 to 10 were prepared in the same manner as Support-1 except for using the following aqueous solutions in place of 1 % sodium nitrite used in preparation of Support-1 and not treating with the CMC aqueous solution.

| | |
|---|---|
| Support-6 | 1 % Sodium nitrite aqueous solution |
| Support-7 | 1 % Potassium nitrite aqueous solution |
| Support-8 | Hot water (80 °C) |
| Support-9 | 1 % Sodium sulfate aqueous solution |
| Support-10 | 1 % Sodium carbonate aqueous solution |

By using the above Supports-6 to 10, Lithographic printing plate samples I-6 to I-10 were obtained in the same manner as in Example 1.

For the samples obtained, evaluations were conducted in the same manner as in Example 1. The results are shown in Table 1.

### Example 2

### Preparation of Supports A-1 and A-2

An aluminum plate (material: 1050, tempering: H16) having a thickness of 0.3 mm was degreased in a 5 % sodium hydroxide aqueous solution at 65 °C for 1 minute, washed, dipped in a 10 % nitric acid aqueous solution at 25 °C for 1 minute, neutralized and then washed. The resulting aluminum plate was electrolytically roughened in a 0.5N hydrochloric acid aqueous solution at 25 °C at an alternate current density of 55 A/dm² for 30 seconds (electrolytical etching in a hydrochloric acid bath, referred to as "Hydrochloric acid EE" in Table 2) and then desmutted in a 5 % sodium hydroxide aqueous solution at 60 °C for 10 seconds. Thereafter, the plate was anodized in a 20 % sulfuric acid solution at 20 °C at a current density of 3 A/dm² for 1 minute, and further sealed for 20 seconds by using hot water of 80 °C.

The aluminum plate having been subjected to the above treatments was dipped in a 1 % sodium nitrite aqueous solution at 90 °C for 1 minute, dipped in a 0.005 % CMC aqueous solution of 90 °C having a pH of 8.5 or 10.0 for 1 minute, washed and dried at 80 °C for 5 minutes to obtain Supports A-1 and A-2.

### Preparation of Support B

Support B was prepared in the same manner as Support A-1 except for using a 1 % CMC aqueous solution having a pH of 8.0 in place of the 0.005 % CMC aqueous solution used in preparation of Support A-1.

### Preparation of Supports C-1 to C-3

Supports C-1 to C-3 were prepared in the same manner as Support A-1 except for using hot water of 90 °C having a pH of 7.0, 8.5 or 10.0 in place of the 0.005 % CMC aqueous solution used in preparation of Support A-1, respectively.

### Preparation of Supports D-1 and D-2

An aluminum plate (material: 1050, tempering: H16) having a thickness of 0.3 mm was degreased in a 5 % sodium hydroxide aqueous solution at 65 °C for 1 minute, washed, dipped in a 10 % nitric acid aqueous solution at 25 °C for 1 minute, neutralized and then washed. The resulting aluminum plate was electrolytically roughened in a 0.3 mole/liter nitric acid aqueous solution at 30 °C at an alternate current density of 50 A/dm² for 30 seconds (electrolytical etching in a nitric acid bath, referred to as "Nitric acid EE" in Table 2) and then desmutted in a 5 % sodium hydroxide aqueous solution at 60 °C for 10 seconds. Thereafter, the plate was anodized in a 20 % sulfuric acid solution at 20 °C at a current density of 3 A/dm² for 1 minute, and further sealed for 20 seconds by using hot water of 80 °C.

On the aluminum plate having been subjected to the above treatments, a 0.05 % sodium formate aqueous solution was coated and dried at 90 °C for 1 minute. Thereafter, the aluminum plate was dipped in a 0.005 % CMC aqueous solution of 90 °C having a pH of 7.0 or 10.0 for 1 minute and washed to prepare Supports D-1 and D-2.

### Preparation of Support E

An aluminum plate (material: 1050, tempering: H16) having a thickness of 0.3 mm was degreased in a 5 % sodium hydroxide aqueous solution at 65 °C for 1 minute, washed, dipped in a 10 % nitric acid aqueous solution at 25 °C for 1 minute, and then washed. The resulting aluminum plate was electrolytically roughened in a 0.3 mole/liter nitric acid aqueous solution at 30 °C at an alternate current density of 50 A/dm² for 30 seconds (electrolytical etching in a nitric acid bath, referred to as "Nitric acid EE" in Table 2) and then desmutted in a 5 % sodium hydroxide aqueous solution at 60 °C for 10 seconds. Thereafter, the plate was anodized in a 20 % sulfuric acid solution at 20 °C at a current density of 3 A/dm² for 1 minute, and further sealed for 20 seconds by using hot water of 80 °C.

The aluminum plate having been subjected to the above treatments was dipped in a 1 % sodium nitrite aqueous solution at 90 °C for 1 minute, dipped in a 0.005 % CMC aqueous solution of 90 °C having a pH of 8.5 for 1 minute, washed and dried at 80 °C for 5 minutes to prepare Support E.

### Preparation of Support F

An aluminum plate (material: 1050, tempering: H16) having a thickness of 0.3 mm was degreased in a 5 % sodium hydroxide aqueous solution at 65 °C for 1 minute, washed, dipped in a 10 % nitric acid aqueous solution at 25 °C for 1 minute, neutralized and then washed. The resulting aluminum plate was grained by a wire brush made of stainless steel (Ra (average roughness): 0.2 µm). After washing, the plate was dipped in a 10 % sodium hydroxide solution at 30 °C for 10 seconds, and the surface thereof was subjected to etching.

Next, the aluminum plate was electrolytically roughened in a 0.5N hydrochloric acid aqueous solution at 25 °C at an alternate current density of 55 A/dm² for 35 seconds (electrolytical etching in a hydrophilic acid bath after brush grinding, referred to as "Multiple" in Table 2) and then desmutted in a 5 % sodium hydroxide aqueous solution at 60 °C for 10 seconds.

Thereafter, the plate was anodized in a 20 % sulfuric acid solution under conditions of a temperature of 20 °C, a current density of 3 A/dm² and a treatment time of 1 minute, and washed.

The aluminum plate having been subjected to the above treatments was dipped in a 1 % sodium nitrite aqueous solution at 90 °C for 1 minute, dipped in a 0.005 % CMC aqueous solution of 90 °C having a pH of 8.5 for 1 minute, washed and dried at 80 °C for 5 minutes to prepare Support F.

### Preparation of Support G (comparison)

An aluminum plate (material: 1050, tempering: H16) having a thickness of 0.3 mm was degreased in a 5 % sodium hydroxide aqueous solution at 65 °C for 1 minute, washed, dipped in a 10 % nitric acid aqueous solution at 25 °C for 1 minute, neutralized and then washed. The resulting aluminum plate was electrolytically roughened in a 0.5N hydrochloric acid aqueous solution at 25 °C at an alternate current density of 55 A/dm² for 30 seconds (electrolytical etching in a hydrochloric acid bath, referred to as "Hydrochloric acid EE" in Table 2) and then desmutted in a 5 % sodium hydroxide aqueous solution at 60 °C for 10 seconds. Thereafter, the plate was anodized in a 20 % sulfuric acid solution at 20 °C at a current density of 3 A/dm² for 1 minute, and further sealed for 20 seconds by using hot water of 80 °C. Thereafter, the plate was dipped in hot water of 80 °C for 1 minutes and dried to prepare Support G.

On Supports A-1 to G prepared as described above, a light-sensitive composition having the following composition was coated by using a wire bar, respectively, and dried at 80 °C for 2 minutes to prepare Light-sensitive lithographic printing plates A-1 to G. The coated film thickness was 2.2 g/m².

### (Composition of light-sensitive composition coating solution)

| | |
|---|---|
| o-Quinonediazide compound (a compound in which 30 mole % of an OH group of a pyrogallol/acetone polycondensed resin having a weight average molecular weight of 2000 is esterified with 1,2-naphthoquinone-5-sulfonyl chloride) | 3.54 g |
| Phenol-cresol resin (a novolak resin having a composition of phenol/m-cresol/p-cresol = 20/48/32 (molar ratio) and a weight average molecular weight of 7000) | 9.1 g |
| Polyethylene glycol #2000 (trade name, produced by Wako Junyaku K.K.) | 0.13 g |
| Victoria Pure Blue BOH (trade name, produced by Hodogaya Kagaku K.K.) | 0.11 g |
| 2-Trichloromethyl-5-(p-methoxystyryl-1,3,4-oxadiazole | 0.13 g |
| Ethylene glycol monomethyl ether | 87.0 g |

The respective light-sensitive lithographic printing plate samples A-1 to G obtained were exposed at 8 mW/cm² for 60 seconds by using a 4 kw metal halide lamp, and developed at 25 °C for 30 seconds by using a 5-fold diluted solution of a developing solution SDR-1 (trade name, produced by Konica Corporation) to prepare Lithographic printing plate samples A-1 to G. Fingers were pressed against the respective lithographic printing plate samples for 5 seconds, and the samples were dried at 55 °C for 20 minutes. Thereafter, printing was carried out by a printing machine Heidelberg GTO (trade name, produced by Heidelberger Druckinaschinen AG (Germany)), stain caused by fingerprint marks and reproducibility of 90 % dot were confirmed. Printing was continued until inking failure was caused at a solid portion of an image portion, and press life was also examined. Also, for the respective samples, the dyeing test by Orange II (trade name, produced by Wako Junyaku K.K.) was conducted. The results are shown in Table 2.

### Evaluation standard of stain caused by fingerprint marks

- ○:: Not inked on fingerprint marks.
- Δ:: Slight inking is observed.
- X:: Apparent inking was formed on marks made by pressing.

### Entanglement of plain dots (90 % dot)

- ○:: Dots are reproduced completely.
- Δ:: Dots are slightly defaced.
- X:: Most of dots are defaced.

As described above in detail, the present invention can provide a light-sensitive lithographic printing plate in which press life is excellent, stain at a non-image portion can be prevented, printing stain caused by fingerprint marks or the like can be prevented and loss of printing papers at the beginning of printing can be reduced.

## Claims

1. A light-sensitive lithographic printing plate which comprises a support being treated by a process comprising steps of neutralizing electric charge of a surface of a pre-treated support; and treating said neutralized support with a hydrophilic polymer aqueous solution, and a light-sensitive layer provided on the support.

2. The plate of Claim 1 wherein the hydrophilic polymer aqueous solution is a solution containing 1 % by weight or less of a hydrophilic polymer and having a pH value of 9 or less and a temperature of 60 °C or higher.

3. The plate of Claim 1 wherein the hydrophilic polymer is a polymer selected from the group consisting of polyacrylic acid, polyacrylamide, polyvinyl alcohol, polyhydroxyethyl acrylate, polyvinyl pyrrolidone, polyethyleneimine, diacryldimethyl ammonium chloride, polyvinylimidazoline, polyalkylaminoethyl acrylate, polyethylene glycol polyoxyethylene, polypropylene glycol, ethylenediamine, hexaethylenediamine, a polyurethane resin, a polyhydroxymethyl urea, a polyhydroxymethyl melamine resin, a soluble starch, carboxymethyl cellulose, hydroxyethyl cellulose, guar gum, tragacanth gum, xanthane gum, sodium alginate and gelatin.

4. The plate of Claim 1 wherein said neutralized support is obtained by treating with nitrous acid and/or a nitrite.

5. The plate of Claim 1 wherein said neutralized support is obtained by treating with a carboxylate represented by any of the following formulae:
(R¹COO)ₙX¹ (I)
wherein n represents 1 or 2; when n is 1, R¹ represents a hydrogen atom, an aliphatic hydrocarbon group having 1 to 10 carbon atoms, an alicyclic hydrocarbon group or an aromatic hydrocarbon group and X¹ represents NH₄⁺ or an alkali metal ion; and when n is 2, R¹s may be the same or different and each represent a hydrogen atom, an aliphatic hydrocarbon group having 1 to 10 carbon atoms, an alicyclic hydrocarbon group or an aromatic hydrocarbon group and X¹ represents a monovalent or divalent metal ion selected from the group consisting of metal ions of the Ia (excluding a hydrogen ion), IIa, VIIa, VIII, IIb and IVb groups of the periodic table, wherein R² represents a direct bond, or a divalent aliphatic hydrocarbon group having 1 to 10 carbon atoms, a divalent alicyclic hydrocarbon group or a divalent aromatic hydrocarbon group; and X² and X³ may be the same or different and each represent NH₄⁺ or an alkali metal ion, or a monovalent or divalent metal ion selected from the group consisting of metal ions of the Ia (excluding a hydrogen ion), IIa, VIIa, VIII, IIb and IVb groups of the periodic table,
R³(COO)₂X⁴ (III)
wherein R³ represents a direct bond, or a divalent aliphatic hydrocarbon group having 1 to 10 carbon atoms, alicyclic hydrocarbon group or aromatic group; and X⁴ represents a monovalent or divalent metal ion selected from the group consisting of metal ions of the Ia (excluding a hydrogen ion), IIa, VIIa, VIII, IIb and IVb groups of the periodic table.

6. The plate of Claim 5 wherein R¹ represents a hydrogen atom or an alkyl group having 1 to 4 carbon atoms; X¹ represents NH₄⁺, an alkali metal ion of sodium, potassium or lithium, or a monovalent or divalent metal ion of calcium, barium, magnesium, zinc, manganese, nickel, strontium or lead; R² represents a direct bond or an alkylene group or phenylene group having 1 to 4 carbon atoms; X² and X³ each represent a hydrogen atom, NH₄⁺ or an alkali metal ion of sodium, potassium or lithium; R³ represents a direct bond or an alkylene group or phenylene group having 1 to 4 carbon atoms; and X⁴ represents a monovalent or divalent metal ion of calcium, barium, magnesium, zinc, manganese, nickel, strontium of lead.

7. The plate of Claim 4 wherein said neutralized support is treated with hot water before being treated with a hydrophilic polymer aqueous solution.

8. The plate of Claim 7 wherein the hydrophilic polymer aqueous solution is a solution containing 1 % by weight or less of a hydrophilic polymer and having a pH value of 9 or less and a temperature of 60 °C or higher.

9. The plate of Claim 7 wherein the hydrophilic polymer is a polymer selected from the group consisting of polyacrylic acid, polyacrylamide, polyvinyl alcohol, polyhydroxyethyl acrylate, polyvinyl pyrrolidone, polyethyleneimine, diacryldimethyl ammonium chloride, polyvinylimidazoline, polyalkylaminoethyl acrylate, polyethylene glycol polyoxyethylene, polypropylene glycol, ethylenediamine, hexaethylenediamine, a polyurethane resin, a polyhydroxymethyl urea, a polyhydroxymethyl melamine resin, a soluble starch, carboxymethyl cellulose, hydroxyethyl cellulose, guar gum, tragacanth gum, xanthane gum, sodium alginate and gelatin.

10. The plate of Claim 1 wherein the light-sensitive layer is a positive type light-sensitive layer.
